

[54] **PYROTECHNIC DISSEMINATING  
FORMULATION**

2,557,815 6/1951 Wheelwright et al..... 149/83 X  
2,637,678 5/1953 Peer et al..... 167/40

[75] Inventor: **Earl Thomas Niles**, Midland, Mich.

*Primary Examiner*—Benjamin R. Padgett

[73] Assignee: **The Dow Chemical Company**,  
Midland, Mich.

*Assistant Examiner*—E. A. Miller

[22] Filed: **Nov. 21, 1966**

*Attorney, Agent, or Firm*—C. Kenneth Bjork; Lloyd S.  
Jowanovitz

[21] Appl. No.: **596,008**

[57] **ABSTRACT**

[52] U.S. Cl. .... **149/84**; 149/76; 149/83;  
149/109.2

This invention comprises a pyrotechnic disseminating  
composition employing an aminosubstituted thiourea  
compound as a fuel, an inorganic oxidizer, such as al-  
kali metal and ammonium chlorates and perchlorates,  
which readily is combustible at atmospheric pressures  
as oxidizer and effective quantities of an agent to be  
disseminated.

[51] Int. Cl.<sup>2</sup> .... **C06D 3/00**

[58] **Field of Search** .... 149/76, 83, 109, 84, 109.2;  
167/40

**6 Claims, No Drawings**

[56] **References Cited**

UNITED STATES PATENTS

2,557,814 6/1951 Dinsdale et al..... 149/83 X

## PYROTECHNIC DISSEMINATING FORMULATION

This invention relates to pyrotechnic dissemination and more particularly is concerned with disseminating systems based on novel pyrotechnic fuel formulations employing aminosubstituted thioureas as a fuel.

Pyrotechnic disseminating formulations are widely employed for colored smoke production used as a signal or screen, for the distribution of plant growth regulating agents such as pesticides, fumigants, herbicides and the like and for the release and distribution of chemicals used in warfare and law enforcement such as tear gas, psychotomimetic incapacitating agents and the like.

The primary problem in disseminating such signalling and treating materials, hereinafter referred to as agents, by pyrotechnic means is in providing a combustible mixture evolving large quantities of gaseous combustion products which burns at a sufficiently low temperature such that the agent being disseminated is not detrimentally degraded or destroyed. In general, such compositions should provide large volumes of gaseous combustion products while undergoing complete burning at a low burning pressure, e.g. a maximum of about two atmospheres, and a maximum burning temperature of about 800° C. and preferably from about 300° to about 600° C. It is another criterium of operation that the agent to be disseminated must be compatible with the pyrotechnic composition to assure reliability of burning after storage as well as storageability without mix degradation.

Heretofore, pyrotechnic dissemination of smoke dyes, herbicides, chemical warfare materials, tear gas and other like agents has been carried out using compositions wherein substantial amounts of the agent to be disseminated are mixed with "cool burning" fuel-oxidizer combinations which provide copious quantities of water vapor and carbon dioxide as the principal gaseous exhaust products. In these formulations, many times undesirable high percentages of the agent are lost through degradation during the combustion dissemination process.

Empirically, it has been found that a mixture of carbohydrates or sulfur with potassium chlorate in the presence of minor amounts of certain additives, e.g. sodium bicarbonate with sulfur or kaolin with sugar, can be used as a pyrotechnic system for dissemination of colored smoke and chemical warfare agents. These systems can be classified as "cool-burning" only because of the flame quenching additives employed therein. Polyvinyl acetate in dilute solutions has been used with these conventional pyrotechnic compositions to increase their physical strength and ease of consolidation. Such solutions reduce the amount of pressure needed to compact the formulations into a "grain". This is of interest especially with those formulations containing sulfur as compaction of such formulations at high pressure is hazardous in that these compositions during fabrication are prone to ignition. Even when partially compacted, the deflagration borders on detonation with respect to velocity. Oil, as a diluent, has been used to moisten and reduce friction sensitivity in such mixtures. This material, however, undesirably degrades the composition from the standpoint of efficiency of dissemination. Thiourea also has been used as a fuel in such compositions. However, it has not proved to be satisfactory since it shows instability in organic

5 dye systems and has not been found to be compatible with certain chemical warfare agents. Additionally, with some agents, mixes containing thiourea have been found to be very impact sensitive even to the point where these could be dangerous to process and store.

10 Dissemination of agents of the type set forth herein also has been realized using pyrochemical gas producers as the high volume gas source. To illustrate, self-sustained gas producing reactions as realized by the relatively low temperature catalytic decomposition of ammonium nitrate, guanidine nitrate and nitroguanidine utilizing chromates and dichromates as catalysts have been used to disperse benzene hexachloride, DDT and other pesticides. These formulations suffer from 15 the disadvantage that they exhibit relatively low efficiency of dissemination and are not universally applicable.

15 It is a principal object of the present invention to provide a novel pyrotechnic composition for dissemination of smoke dyes, pesticides, chemical warfare and the like agents.

20 It is also an object of the present invention to provide a pyrotechnic formulation which is safe to handle during mixing and other production operations when in admixture with an agent to be disseminated.

25 It is a further object of the present invention to provide a pyrotechnic formulation containing an agent to be disseminated wherein the resultant composition remains stable under prolonged storage even at relatively elevated temperatures of 60° C. or more and which gives high efficiencies of gaseous combustion production and agent dissemination upon use.

30 It is another object of the present invention to provide a pyrotechnic composition suitable for use with a wide variety of agents ordinarily dispersed by pyrotechnic dissemination.

35 It is also an object of the present invention to provide a cool-burning pyrotechnic composition for dissemination of agents which requires no coolant additives.

40 These and other objects and advantages readily will become apparent from the detailed description of the invention presented hereinafter.

45 The present invention comprises a pyrotechnic disseminating composition employing an aminosubstituted thiourea compound as a fuel, inorganic oxidizers which readily are combustible at atmospheric pressures as oxidizer and effective quantities of an agent to be disseminated.

50 More particularly, the present invention comprises from about 6 to about 23 weight per cent of thiourea,



60 (hereinafter designated as TSC), ethylenebis(thiourea),



(coded as EBS), thiocarbohydrazide,



(herein designated as TCH) and dithiobiurea,



(denoted as DTB), from about 20 to about 36 weight per cent of an alkali metal or ammonium chlorate or perchlorate such as, for example, sodium chlorate ( $\text{NaClO}_3$ ), potassium chlorate ( $\text{KClO}_3$ ) or ammonium perchlorate ( $\text{NH}_4\text{ClO}_4$ ), and balance agent to be disseminated. A preferred embodiment of the present invention comprises from about 8 to about 13 weight per cent of a fuel as listed directly hereinbefore, from about 23 to about 30 weight per cent potassium chlorate, and balance agent to be disseminated.

These formulations exhibit a satisfactory burning rate, are cool burning and develop copious quantities of neutral (i.e. substantially non-reactive with agent) gaseous combustion products to provide good agent dissemination. If desired, however, optionally up to about 10 per cent by weight, preferably from about 0.2 to about 2 weight per cent of a combustion catalyst, e.g. chromates, copper salts, platinum, rhodium or iridium metals, ferrocene, metal chromites, ferric oxide and the like can be incorporated into the formulation. Alkali metal chromates, e.g. potassium chromate ( $\text{K}_2\text{CrO}_4$ ) and copper halides, e.g. copper chloride, have been found to be particularly suitable catalysts. The use of the combustion catalyst appears to stabilize the burning rate somewhat and provide more consistent results particularly with the faster burning compositions. This in turn results in somewhat higher efficiencies and aerosol yields.

Agents for dissemination which can be incorporated into the formulation include for example organic dyes such as methylaminoanthraquinone (MAAQ) used for the production of colored smoke, the condensation product of chlorobenzaldehyde and malononitrile commonly employed as a tear gas and hereinafter designated as CS, incapacitating agents which are psychotomimetics such as the classified materials having unclassified U.S. Government code designations BZ and EA-3443, herbicides, fungicides, pesticides and the like.

By "effective quantities" of such agents is meant those amounts whereby a predetermined level of treatment or activity is realized as is understood by one skilled in the art of pyrotechnic dissemination.

The formulations can be fabricated into compacts or grains using techniques and procedures commonly employed in the art. Blends usually are made by mixing the components, placing the resulting substantially

homogeneous mix into a container, compacting the mix in the container and contacting the so-compacted formulation with an ignition system and igniter.

Internal burning grains are prepared by pressing or compacting the blend around a mandrel of predetermined shape and size.

The present novel pyrotechnic disseminating formulation offers the unexpected advantages of safety during mixing with agents that are somewhat hazardous to handle in the presence of sulfur. Also, they provide unexpectedly high stability during storage as well as higher efficiency of dissemination when compared with formulations based on conventional pyrotechnic systems.

15 The following Examples will serve to further illustrate the present invention but are not meant to limit it thereto.

#### EXAMPLE 1

20 For aerosol evaluation, a large number of formulations were prepared by mixing a fuel and catalyst (if catalyst was employed), incorporating an agent into the system followed by oxidizer. The resulting formulation totalling 10 grams, was mixed remotely in a revolving bottle to provide a substantially homogeneous blend. The so-blended pyrotechnic disseminating composition was placed in a small metal can (1.125 inches diameter by 2.25 inches high) and compacted by an applied pressure of about 1500 pounds per square inch. The cover of the can was pierced to provide an 0.25 inch opening. A MIL SPEC No. 508 First Fire and a No. 565 Squib igniter was inserted into the can through this opening and placed in contact with the dissemination formulation.

25 30 35 The pressed grain was ignited and burning characteristics, including ease of ignition, burning time, combustion temperature and pressure were recorded. Additionally, the aerosol yield,

$$(Aerosol yield (\%)) = \frac{\text{Agent in Aerosol Form} \times 100}{\text{Total Weight Composition}}$$

40 and Efficiency,

$$(Efficiency (\%)) = \frac{\text{Agent in Aerosol Form} \times 100}{\text{Agent in Composition}}$$

45 also were measured.

50 55 The results of these studies are summarized in Tables I and II. To aid in the ease of understanding and ready presentation of the results, the operable and optimum composition ranges are shown in Table I. Table II summarizes the burning characteristics and compatibility characteristics exhibited by the compositions of corresponding number in Table I.

Table I

| Comp. No. | Component | Fuel          |               |                |                | KClO <sub>3</sub> Oxidizer |               |                |                | Component           | Agent         |               |                |                | Remarks                         |
|-----------|-----------|---------------|---------------|----------------|----------------|----------------------------|---------------|----------------|----------------|---------------------|---------------|---------------|----------------|----------------|---------------------------------|
|           |           | Operable min. | Operable max. | Preferred min. | Preferred max. | Operable min.              | Operable max. | Preferred min. | Preferred max. |                     | Operable min. | Operable max. | Preferred min. | Preferred max. |                                 |
| 1a        | TSC       | 10            | 17            | —              | —              | 23                         | 29            | —              | —              | MAAQ <sup>(1)</sup> | 60            | —             | —              | —              | System not completely optimized |
| 1b        | TSC       | —             | —             | 10             | 12             | —                          | —             | 28             | 29             | MAAQ <sup>(1)</sup> | —             | —             | 60             | —              | System not optimized            |
| 2         | TCH       | 12            | 19            | —              | —              | 21                         | 28            | —              | —              | MAAQ <sup>(1)</sup> | 60            | —             | —              | —              |                                 |
| 3a        | EBS       | 7             | 17            | —              | —              | 25                         | 36            | —              | —              | MAAQ <sup>(2)</sup> | 50            | 60            | —              | —              | System not completely optimized |
| 3b        | EBS       | —             | —             | 9              | 12             | —                          | —             | 28             | 30             | MAAQ <sup>(2)</sup> | —             | —             | —              | 60             | System not completely optimized |
| 4a        | EBS       | 6             | 18            | —              | —              | 20                         | 33            | —              | —              | CS                  | 56            | 65            | —              | —              |                                 |

Table I-continued

| Comp. No. | Component | Fuel          |               |                                |                                | KClO <sub>3</sub> |               |                                |                                | Component           | Agent         |               |                                |                                | Remarks                         |
|-----------|-----------|---------------|---------------|--------------------------------|--------------------------------|-------------------|---------------|--------------------------------|--------------------------------|---------------------|---------------|---------------|--------------------------------|--------------------------------|---------------------------------|
|           |           | Operable min. | Operable max. | Parts by Weight Preferred min. | Parts by Weight Preferred max. | Operable min.     | Operable max. | Parts by Weight Preferred min. | Parts by Weight Preferred max. |                     | Operable min. | Operable max. | Parts by Weight Preferred min. | Parts by Weight Preferred max. |                                 |
| 4b        | EBS       | —             | —             | 8                              | 12                             | —                 | —             | 23                             | 25                             | CS                  | —             | —             | 64                             | 68                             | System not completely optimized |
| 5a        | DTB       | 10            | 23            | —                              | —                              | 26                | 33            | —                              | —                              | MAAQ <sup>(2)</sup> | 50            | 60            | —                              | —                              | System not completely optimized |
| 5b        | DTB       | —             | —             | 10                             | 13                             | —                 | —             | 27                             | 30                             | MAAQ <sup>(2)</sup> | —             | —             | —                              | 60                             | System not completely optimized |

<sup>(1)</sup>Methylaminoanthraquinone having blended therewith 15 percent by weight dextrin<sup>(2)</sup>Methylaminoanthraquinone

Table II

| Comp. No. | Burning Time Range (sec.) | Combustion Temperature range (°C.) | Combustion Pressure Range | Ignition Characteristics | Aerosol Yield Range (%) | Efficiency Range (%) | Compatibility |       |          |                             |         |
|-----------|---------------------------|------------------------------------|---------------------------|--------------------------|-------------------------|----------------------|---------------|-------|----------|-----------------------------|---------|
|           |                           |                                    |                           |                          |                         |                      | Impact        | Spark | Friction | Surveillance <sup>(1)</sup> | General |
| 1a        | 12-18                     | 390                                | G                         | G                        | G to M                  | G to M               | G             | G     | G        | G                           | G       |
| 1b        | 12-16                     | 390                                | G                         | G                        | 35-38                   | 59-63                | G             | G     | G        | G                           | G       |
| 2         | 10-22                     | 350-510                            | L to G                    | G                        | M to G                  | M to G               | G             | G     | G        | G                           | G       |
| 3a        | 7-12                      | 380-500                            | P to G                    | P to G                   | 28-42                   | 56-69                | G             | G     | G        | G                           | G       |
| 3b        | 7-9                       | 425-450                            | G                         | G                        | 38-42                   | 63-69                | G             | G     | G        | G                           | G       |
| 4a        | 6-32                      | 350-540                            | M to G                    | G                        | 26-54                   | 43-82                | G             | G     | G        | G                           | G       |
| 4b        | 8-10                      | 350-475                            | G                         | G                        | 48-54                   | 71-82                | G             | G     | G        | G                           | G       |
| 5a        | 7-13                      | 350-390                            | G                         | G                        | 27-37                   | 50-62                | G             | G     | G        | G                           | G       |
| 5b        | 9-11                      | 375-390                            | G                         | G                        | 36-37                   | 60-62                | G             | G     | G        | G                           | G       |

P=Poor, L=Low M=Medium, G=Good (Based on Poor as minimum acceptable performance for use in agent dissemination)

<sup>(1)</sup>Formulation compatibility after long term (9-12 weeks) storage at about 70° C.

## EXAMPLE 2

Following the same procedure as set forth in Example 1, a number of specific formulations were blended and pressed into 10 gram grains for aerosol evaluation. Additionally, several disseminating formulations were fabricated into internal burning grains by pressing a substantially homogeneous mixture around a  $\frac{1}{8}$  inch mandrel.

These were ignited using the igniter system described in Example 1 and the combustion characteristics noted.

The composition of the formulations and their combustion characteristics are summarized in Table III.

KClO<sub>3</sub> and CS or BZ agent. These were tested for resistance to impact, spark, friction and given a surveillance test as described for Example 1. In all of these studies, these were rated as Good. The general compatibility exhibited by each of these formulations also was Good.

## EXAMPLE 4

Following the procedure set forth in Example 1, dithiobiurea, potassium chlorate and CS agent, with and without potassium chromate catalyst, were fabricated into end burning pyrotechnic disseminating grains. These were ignited and the combustion characteristics measured.

Table III

| Run No. | Fuel type | Formulation |                     | Agent type          | Burning Time (sec.) | Combustion Temperature °C. | Combustion Characteristics |              |             | REMARKS                                                                                       |
|---------|-----------|-------------|---------------------|---------------------|---------------------|----------------------------|----------------------------|--------------|-------------|-----------------------------------------------------------------------------------------------|
|         |           | Fuel %      | KClO <sub>3</sub> % |                     |                     |                            | Aerosol Yield %            | Efficiency % |             |                                                                                               |
| 1       | EBS       | 10.3        | 29.7                | MAAQ                | 60.0                | 7                          | ~ 470                      | 41           | 68          |                                                                                               |
| 2       | EBS       | 12.0        | 23.0                | CS                  | 65.0                | 10-11                      | ~ 445                      | 46.5-53.5    | 72-82       |                                                                                               |
| 3       | TSC       | 12.0        | 28.0                | MAAQ <sup>(1)</sup> | 60.0                | 10.5                       | ~ 430                      | 37.5         | 63          |                                                                                               |
| 4       | TCH       | 14.7        | 25.3                | MAAQ <sup>(1)</sup> | 60.0                | 12                         | ~ 500                      | not sampled  | not sampled | Qualitative evaluation as determined visually indicated good aerosol yield and efficiency     |
| 5       | DTB       | 12.8        | 27.2                | MAAQ                | 60.0                | 9                          | ~ 380                      | 37           | 61.5        |                                                                                               |
| 6       | EBS       | 19.0        | 31.0                | BZ                  | 60.0                | 20                         | not recorded               | not sampled  | not sampled | Grain was cool burning and qualitatively shown to burn with good aerosol yield and efficiency |

<sup>(1)</sup>15% by weight dextrin blended with MAAQ

## EXAMPLE 3

Following the procedure set forth in Example 1, a number of pyrotechnic disseminating formulations, within the composition ranges set forth herein, were fabricated from thiosemicarbazide, thiocarbohydrazide, ethylenebis(thiosemicarbazide) and dithiobiurea,

65 Additionally, the grains were tested for compatibility by evaluating their resistance to impact, spark, friction, surveillance. Their general compatibility also was noted. Each composition rated as Good in all of the compatibility tests.

Table IV presents the formulation compositions and combustion characteristics.

Table IV

| Run No. | DTB<br>Fuel<br>% | Formulation            |                  |                                                  | Burning<br>Time<br>(sec.) | Combustion Characteristics         |                       |                 |
|---------|------------------|------------------------|------------------|--------------------------------------------------|---------------------------|------------------------------------|-----------------------|-----------------|
|         |                  | KClO <sub>3</sub><br>% | CS<br>Agent<br>% | K <sub>2</sub> CrO <sub>4</sub><br>Catalyst<br>% |                           | Combustion<br>Temperature<br>(°C.) | Aerosol<br>Yield<br>% | Efficiency<br>% |
| 1       | 11.5             | 28.5                   | 60               | —                                                | 19                        | 380-400                            | 41.5                  | 69.2            |
| 2       | 11.0             | 28.0                   | 60               | 1                                                | 12.5                      | 380                                | 49.5                  | 82.5            |
| 3       | 10.5             | 27.5                   | 60               | 2                                                | 12                        | 300-340                            | 51.0                  | 85.0            |

In a manner similar to that described for the foregoing experiments, pyrotechnic disseminating formulations having herbicides, fungicides, and the like pesticides incorporated therein can be prepared using the fuel and oxidizer system disclosed herein. It is to be understood that combustion catalysts, e.g. potassium chromate, copper chloride, platinum, rhodium, iridium, sodium dichromate, chromic acid (CrO<sub>3</sub>), copper chromite, ferric oxide and the like, as disclosed herein alternatively can be utilized in these compositions.

Various modifications can be made in the present invention without departing from the spirit or scope thereof for it is understood that I limit myself only as defined in the appended claims.

I claim:

1. A pyrotechnic disseminating formulation comprising

- a. from about 6 to about 23 weight per cent of an aminosubstituted thiourea as fuel,
- b. from about 20 to about 36 weight per cent of a member selected from the group consisting of alkali metal and ammonium chlorates and perchlorates as oxidizer, and

c. balance an agent to be disseminated selected from the group consisting of smoke producing organic dyes, tear gas, herbicides, fungicides, pesticides, and psychotomimetic incapacitating agents.

2. The composition as defined in claim 1 wherein the fuel is a member selected from the group consisting of thiosemicarbazide, ethylenebis (thiosemicarbazide), thiocarbohydrazide and dithiobiurea and the oxidizer is potassium chlorate.

3. The composition as defined in claim 2 wherein the fuel ranges from about 8 to about 13 weight per cent and the oxidizer ranges from about 23 to about 30 weight per cent.

4. The composition as defined in claim 1 and including up to about 10 weight per cent of a combustion catalyst.

5. The composition as defined in claim 1 and including from about 0.2 to about 2 weight per cent of a combustion catalyst.

6. The composition as defined in claim 5 wherein the combustion catalyst is potassium chromate.

\* \* \* \* \*

35

40

45

50

55

60

65